

## UNITED STATES PATENT OFFICE

JULIUS HYMAN, OF CHICAGO, ILLINOIS, ASSIGNOR TO THE PURE OIL COMPANY, OF CHICAGO, ILLINOIS, A CORPORATION OF OHIO

## ARTIFICIALLY COLORED MOTOR FUEL

No Drawing.

Application filed September 25, 1929. Serial No. 395,198.

The present invention relates broadly to hydrocarbon fuels for internal combustion engines, and in its more limited aspects to engine fuels, such as gasoline, which contain artificial coloring matter. It is the principal object of the present invention to provide an artificially colored motor fuel wherein provision is made for causing the fuel to retain its desired appearance or color values for extended periods of time. 5

There is in common practice at present among refineries and distributors of gasoline the use of oil soluble coloring materials, such as aniline dyes, as ingredients in some of the 15 gasolines or motor fuels now obtainable on the market. Usually, such colors have as their purpose the identification of the gasoline in question.

Due to differences in coloring power, some 20 colors or dyes are more advantageously used than others. Substantially all oil colors or dyes, however, lose their coloring power to a greater or lesser extent upon exposure in solution, and, generally, this decrease in coloring power is known as "bleaching". For example, sunlight appears to be the most active of the natural bleaching catalysts or agents, although materials present in the atmosphere, such as ozone, are believed to exert similar, although not so pronounced, effects. 25

I have found that certain materials, added to the gasoline or other motor fuel spirit, will retard the bleaching of oil soluble colors 30 to a greater or less degree, depending on the nature and relative amounts present of the anti-bleach and dye, the nature of the motor spirit and the intensity of the bleaching catalyst. I have found further, that these 35 anti-bleaches or color stabilizing agents are the same materials which will reduce the activity of organic per-acids, either by reduction to the normal acid or by salt formation.

Among the anti-bleach materials above 40 described are, on the one hand, reducing compounds such as catechol and many other hydroxy- and amino-derivatives of benzol and, on the other hand, ammonia and its derivatives. Inasmuch as only small amounts of 45 these materials need be added to the motor

fuel for complete effectiveness, the additional cost is very slight and marked advantages obtained, especially where the motor fuel or gasoline is exposed to light and air in, for example, the measuring cylinders of filling station or garage pumps. 55

As the amount of anti-bleach material used will be determined largely by its cost and solubility, it is not considered necessary or advisable to place herein any specific limitations 60 on the amount of the material to be used, nor is the invention limited in its scope to the specific anti-bleach materials above mentioned, since the invention includes within its purview the employment of any materials 65 which reduce the activity of organic per-acids and any desired proportion of the materials to the liquids under treatment to obtain the ends specified.

Having thus described this invention, what 70 I claim is:

1. A fuel composed essentially of volatile hydrocarbons for use in internal combustion engines containing a soluble coloring matter normally tending to lose its coloring power 75 under conditions of storage and an anti-agent tending to stabilize such color deterioration.

2. The method of stabilizing the characteristics of artificially colored hydrocarbon motor fuel oils of the type containing soluble coloring matter and which tend to deteriorate in color upon exposure to light and air, which comprises adding thereto prior to such deterioration a small proportion of a hydroxy-aromatic compound sufficient to reduce the 85 activity of organic per-acids present in said oil and inhibit loss of the desired color thereof. 80

3. The process of inhibiting loss of color in artificially dyed gasolines containing soluble unstable coloring compounds normally tending to fade upon storage, which comprises mixing therewith and dissolving therein a hydroxy-aromatic compound in sufficient quantities to substantially inhibit bleaching 90 or loss of desired color of the gasoline. 95

4. A gasoline for use in internal combustion engines, said gasoline having a non-anti-oxidant coloring substance therein, said coloring substance being unstable and an anti-ox-

idant hydroxy-benzol in sufficient amount to stabilize said coloring substance.

5. A fuel composed essentially of volatile hydrocarbons for use in internal combustion engines containing a soluble coloring matter normally tending to fade upon storage and a color stabilizing agent comprising catechol.

6. A fuel composed essentially of volatile hydrocarbons for use in internal combustion engines containing a soluble coloring matter normally tending to fade upon storage and a color stabilizing agent composed of amino derivatives.

7. A gasoline for use in internal combustion engines, said gasoline having a non-antioxidant coloring substance therein, said coloring substance being unstable and an antioxidant amino-benzol in sufficient amount to stabilize said coloring substance.

20 8. A fuel composed essentially of volatile hydrocarbons for use in internal combustion engines containing a soluble coloring matter normally tending to fade upon storage and a color stabilizing agent comprising ammonia.

In testimony whereof I affix my signature.  
JULIUS HYMAN.

30

35

40

45

50

55

60

65